

## UNITED STATES PATENT OFFICE.

HUGO SCHNEIDER, OF HASTINGS, NEW YORK.

## TOILET-ARTICLE FILLING COMPOSITION.

No Drawing.

Application filed May 10, 1920. Serial No. 380,409.

*To all whom it may concern:*

Be it known that I, HUGO SCHNEIDER, a citizen of the United States, and resident of Hastings, in the county of Westchester and State of New York, have invented certain new and useful Improvements in Toilet-Article Filling Composition, of which the following is a specification.

My invention relates to the manufacture of filled toilet articles, and is especially directed to an improvement in the composition employed as a filler therefor.

A large variety of toilet articles, such as hand mirrors, brushes, combs, manicure implements, various types of containers, and the like, are manufactured wholly or in part from celluloid, pyroxilin compounds, or similar substances. In order to avoid the expense of manufacturing such articles from solid stock, they have heretofore been constructed from a hollow shell of suitable material filled with a composition providing proper strength and solidity.

However, the fillers heretofore employed have each been open to one or more serious objections which rendered them relatively undesirable. One source of trouble with such fillers has been the tendency to shrink after being positioned in the shell, producing weakened spots in which the shell is unsupported, and also developing a tendency to rattle.

Another defect has been the relative brittleness of the filler, causing it to crack and rattle, which not only weakens the structure of the article, but also produces an article which is unpleasant to use, reducing the saleability thereof. Other fillers have not been of proper weight, and toilet articles of the nature indicated which are either too heavy or too light are inconvenient to use and much less desirable.

While filled toilet articles may be manufactured in different ways, one highly efficient process includes the construction of a hollow shell and the subsequent insertion of the filler therein by pouring it into a suitable aperture in the shell. Consequently, a filler which is to be employed in manufacturing filled articles by this process should not only avoid the defects above outlined, but must also possess the faculty of flowing readily into all parts of the interior of a hollow shell, and of hardening in place therein without shrinking, cracking, becoming

ing brittle, or losing its substantially homogeneous consistency.

It furthermore must be of such a nature as to have no harmful effects upon the material of which the shell is composed.

The composition which I have invented is suitable for use with mirrors or other toilet articles of the type shown in my copending application No. 299,299, and is located therein in the same way.

I have also found that a suitable filler of this nature should remain substantially firm at temperatures above the ordinary, such as those encountered in hot climates, as well as those produced in the course of manufacture, as by buffing, grinding or otherwise operating on the shell in finishing the article.

I have found that the characteristics above outlined are possessed by a composition including a suitable intermixture of wax and a resinous or gummy substance, preferably combined with an inert filler or weighting material, such as finely powdered mineral matter. Any of the many forms of wax are suitable for my purpose, including both those of animal origin, such as stearine, tallow, beeswax, and the like, and those of mineral origin, such as commercial paraffin. I likewise may employ any of the various substances of a gummy, resinous or rosin-like nature, a great variety of which is well known to those skilled in the art. Examples of such substances are rosin, resin and gum tragacanth.

By combining the wax and gummy material in suitable proportions, I provide a substance which may be melted at a convenient temperature for pouring into a hollow toilet article, and which hardens without shrinking or becoming brittle. Furthermore, such mixture while solid may be of such a consistency that if desired it may be cut into suitable filling shapes and the shells placed thereon, this method also being employed for the manufacture of articles of the type described. Such a filler possesses sufficient hardness to support a relatively thin shell at all points, but retains a certain slight resiliency which prevents cracking when the article is dropped or subjected to blows.

I have also found it desirable to include with the wax and the gummy substance a suitable proportion of the weighting substance or filler, whose function is primarily

60

65

70

75

80

85

90

95

100

105

110

to give proper body or weight to the composition, although it also contributes a certain amount of strength thereto. For this purpose, I may employ a variety of materials, preferably in finely powdered form, and including the various mineral or rock-forming substances. Examples of materials which I have found suitable for this purpose are marble dust and terra alba, the primary characteristics required being the ability to mix readily with the other ingredients to form a homogeneous mass which will not settle out into its component parts before it has a chance to harden and after insertion in the filled article.

The proportions employed vary somewhat, depending upon the exact substances used. Through experiment, I have found that the best results are obtained by employing a mixture of paraffin with rosin, using either marble dust or terra alba as the filler. With a composition of this type, the employment of too much wax will result in a soft product which will not offer the proper support to the shell, and which will be effected by the heat of torrid climates as well as by heat generated in finishing the article. Furthermore, such an excess in wax will tend to cause such wax to gather at the surface of the composition immediately under the article shell during filling, causing soft spots not only readily affected by heat, but directly liable to deformation by pressure. On the other hand, an excess of rosin will produce a brittle filler which is readily cracked by blows and therefore undesirable from a commercial standpoint.

I have ascertained that a composition having the desired characteristics can be produced by mixing thoroughly the paraffin and rosin in the proportion of twenty pounds of wax to fifteen pounds of rosin. However, it will be apparent that these proportions will vary somewhat depending upon the type of wax and of gum employed. A smaller proportion of the harder gums will produce a composition of equal hardness to that described, and a small proportion of softer waxes will likewise produce the same effect, the characteristics of the various gums and waxes being well known to those skilled in the art, and the relative proportions employed being determined primarily by the relative hardness and melting point of the ingredients. The amount of weighting material or filler, such as marble dust or terra alba, is determined solely by the weight of the article which is desired, and is therefore largely a matter of taste and the specific toilet article in which the filler is used. I have found that when twenty pounds of wax and fifteen pounds of rosin are used, twenty pounds of marble dust produces a composition having the proper weight for mirror backs of the type described in my said co-

pending application, but such proportion of marble dust is illustrative only.

The various ingredients may be compounded in any desired way, preferably by melting the wax and gummy substance and mixing them together with the powdered weighting material. The mixture may then be poured into a suitable hollow shell and allowed to harden therein, or it may be molded or rolled while soft and plastic into suitable form, such as flat sheets, from which filler sections of suitable contour may be cut. Likewise, the halves of a hollow shell may be pressed into opposite sides of a sheet of suitable thickness to produce the filled article, preferably while the sheet is sufficiently warm to be plastic.

While I have referred to one of my ingredients as a gummy substance or gum, it is to be understood that this expression is not confined purely to the resinous class of gums, but includes rosin and other substances having the physical characteristics generally and popularly included within the term "gum." Furthermore, I have not used the term "wax" in a strictly chemical sense, but intend it to include the various substances, both of mineral and of animal or plant origin, having the physical characteristics ordinarily and popularly indicated by the term "wax."

Likewise, I do not intend to limit myself to a specific powdered weighting material or filler, as such substance has a very slight effect on the composition, and a very wide variety of substances suitable for the purpose are well known to those skilled in the art, and may be interchangeably used, the only requisite being the capacity to form a homogeneous mixture and relative inertness toward the other components.

I claim:

1. A composition adapted for use as a filler for toilet articles, comprising in combination a wax and a gum in the proportion of approximately 15 pounds of gum to 20 pounds of wax, thoroughly intermixed to produce a substance relatively hard, but not brittle, under any climatic conditions.

2. A composition adapted for use as a filler for toilet articles, formed by combining a wax, a gum, and a finely divided relatively inert filler in thoroughly intermixed relation to produce a substance relatively hard, but not brittle, under any climatic conditions.

3. A composition adapted for use as a filler for toilet articles, formed by combining a wax, a gum, and a finely divided relatively inert mineral substance in thoroughly intermixed relation to produce a substance relatively hard, but not brittle, under any climatic conditions.

4. A composition adapted for use as a filler for toilet articles, comprising a wax, a finely divided relatively inert mineral

filler, and a gum thoroughly intermingled in the proportions of 20 pounds of wax, 20 pounds of filler, and from 8 to 35 pounds of gum, to produce a substance relatively hard, 5 but not brittle, under any climatic conditions.

5. A composition adapted for use as a filler for toilet articles, comprising a wax, a finely divided relatively inert mineral filler, 10 and a gum thoroughly intermingled in the

proportions of 20 pounds of wax, 20 pounds of filler, and approximately 15 pounds of gum, to produce a substance relatively hard, but not brittle, under any climatic conditions.

Signed at Hastings, in the county of Westchester and State of New York this 8th day of May, A. D. 1920.

15  
HUGO SCHNEIDER.